

## 1

3,827,952

**ALUMINUM ALLOY ARCHITECTURAL SHEET PRODUCT AND METHOD FOR PRODUCING**  
Edmund C. Franz, Pittsburgh, Pa., assignor to Aluminum Company of America, Pittsburgh, Pa.  
No Drawing. Filed Sept. 20, 1972, Ser. No. 290,653  
5 Int. Cl. C23b 9/02; C22f 1/04  
U.S. Cl. 204—29

12 Claims

**ABSTRACT OF THE DISCLOSURE**

Improved aluminum alloy sheet containing silicon, copper and chromium in controlled amounts and having a high purity aluminum base is capable of producing integrally colored anodic coatings and is highly formable. The integral coatings can range in color from gold through bronze shades to a true black. The alloy has improved corrosion resistance and is highly suited for architectural applications. The production of the alloy sheet product includes a high temperature homogenization together with controlled hot and warm rolling practices to achieve a fine internal structure.

**Background of the Invention**

Aluminum sheet and other products have found wide acceptance in the architectural field where they form substantial portions or even all of the exterior of several high-rise or other type buildings. Especially useful are those aluminum products which, when anodized, achieve an integrally colored oxide coating. The integral color is preferable to a dyed or otherwise imparted color since it is more durable and has aesthetic advantages with respect to the depth of the color. However, aluminum alloy sheet products capable of economical and rapid color development in anodizing baths together with good forming characteristics and good corrosion resistance have been difficult to achieve. For instance, some products can achieve a desired color, for instance, a black color, but are not readily formed as by bending into the shapes desired for a given curtain wall design. Others that can be bent or otherwise formed tend to develop incipient cracks, folds or checking through the bend radius which disrupts the integrity of the anodic coating in this area. Moreover, the colored anodic coating itself tends to exhibit a crackled or checked appearance in that the anodic coating appears much rougher through the radius of the bend as opposed to its appearance on flat portions. This problem seems tied somehow to the hot rolling employed to reduce the thickness of the ingot or starting stock. However, economic production of a sheet product requires a substantial amount of hot rolling using existing or conventional equipment. Another problem encountered with many aluminum alloy products in architectural applications is caused by atmospheric pollution which can corrode the sheet product even when anodized and detract from its aesthetic qualities. For instance, certain atmospheric pollutants can cause an integral black color on an aluminum alloy sheet or plate product to exhibit a blue smudgy appearance which can be objectionable.

**DESCRIPTION**

In accordance with the invention an improved aluminum architectural sheet product is provided which has high resistance to corrosion, is readily formed by bending or other working operations to produce desired shapes which when anodized are substantially free from any crackling or checking in areas where the sheet is bent. The sheet is capable of producing an integral black color within 30 minutes employing existing commercially accepted anodizing methods. The sheet is also capable of achieving gold or other colors by altering the anodizing conditions.

## 2

The improved sheet is fashioned from an improved alloy consisting essentially of 0.4 to 0.6% copper, 0.1 to 0.25% chromium, 0.08 to 0.18% silicon, the balance being aluminum and not more than the following amounts of other elements and impurities: iron 0.3%, manganese 0.05%, zinc 0.05%, titanium 0.05%, magnesium 0.1%, all others being limited to 0.05% each and a total of 0.1%. Further the total amount of all impurities not including iron, should not exceed 0.2%. While magnesium has been described as an impurity, one preferred embodiment of the invention contemplates controlled additions of magnesium within the range of up to 0.1%, the preferred minimum for magnesium being 0.005% and the preferred maximum being 0.05%. Within these limits magnesium confers an advantage on the improved sheet with respect to reducing any tendency for structural streaking.

The improved method for producing the architectural sheet product contemplates providing a body of the alloy described above and homogenizing it at a sufficiently high temperature to dissolve the chromium and copper containing phases after which the metal is hot-warm rolled at controlled temperature levels to produce a sheet product. The sheet product so produced can, if desired, be further worked by cold rolling which can advantageously strengthen the sheet by strain hardening and the cold rolling can be preceded by an anneal. If ease of forming is important any cold rolling can be followed by an anneal.

30 The alloy is produced as an ingot by any of the means conventionally employed although continuous casting is preferred. Economical production requires starting with an ingot of substantial thickness, at least 8 inches and preferably 10 inches or more in thickness, for instance 12 inches or even greater. However, the hot rolling normally required in fabricating a rolled product from starting stock of this size seems to cause the bend appearance problem discussed above regardless of subsequent operations or treatments. However, as explained below certain special controls in accordance with the present improvement alleviates this condition thereby enabling economical production of an improved architectural sheet product.

45 The ingot is homogenized by heating to a temperature of 1000° to 1150° F., preferably 1050° to 1100° F., for a period typically ranging from about 4 to 20 hours or more. This assures solution of the copper and chromium containing phases and further spherodizes the constituent phases such as Al-Fe-Si and Al-Fe-Cr constituents. The ingot is then cooled to room temperature or cooled to about 800° F. for rolling. It is preferred that any cooling be fairly rapid as by cooling in open air as opposed to furnace cooling and the improved method favors such rapid cooling rates as are commensurate with open air cooling.

55 The homogenized ingot is scalped and rolled at controlled temperatures ranging from 300° to 800° F. In accordance with the invention it has been found that the initial hot rolling passes impart certain characteristics to the grain structure of the rolling stock which are reflected in the final product regardless of the subsequent fabrication steps even if they include drastic cold reductions. It has been found that the improved sheet alloy described above cannot sustain working operations above temperatures of about 850° F. without exhibiting appearance problems in bend areas. This effect seems connected with the fact that conventional hot working operations at temperatures of 850° to 950° F. can elongate the grains considerably without any significant amount of grain fragmentation occurring. While the grain elongation effect is not of special significance it is especially important that

the very first passes produce at least some significant amount of grain fragmentation across the long transverse direction or dimension as it is this which avoids the development of any banded grain structure. The long transverse direction is that corresponding to the sheet width, that is normal to the sheet length and to the sheet thickness. It has been found that the first hot rolling passes set the pattern for this effect which pattern exerts a strong influence on the final product regardless of subsequent fabricating operations, even drastic cold rolling and the drastic grain fragmentation associated therewith. In accordance with the invention it is important that rolling operations at temperatures of over 800° F. be substantially avoided since they produce grain elongation without sufficient grain fragmentation along the long transverse dimension. Accordingly, the invention contemplates avoiding such operations at temperatures over 800° F. and instead contemplates hot rolling at rolling mill entrance temperatures of 600° to 800° F., preferably 700° to 800° F. That is, the ingot or rolling stock is cooled to or reheated to provide a substantially uniform metal temperature of 600° or 700° to 800° F. as the metal enters the hot rolling mill. The metal can, however, be brought to a higher temperature, say 825° or 850° or even 900° F. prior to rolling, so long as it is cooled to substantially not over 800° F. as it enters the rolling operations.

The invention contemplates substantial reductions at elevated but controlled temperatures which can economically be carried out in hot and continuous mills. Accordingly, the rolling stock is hot-warm rolled at temperatures between the entrance temperature of not over 800° F. down to temperatures of 300° F. or higher. It is preferred that temperatures during the hot-warm rolling do not fall below 375° F. and preferably not below 450° F. The extent of the rolling reductions at the controlled elevated temperatures should amount to at least 40% of the thickness of the starting stock and preferably at least 80%, and it is preferred that the reductions proceed without reheating the metal to compensate for heat lost in the rolling operation. These reductions at these controlled temperatures result in a grain structure which, while somewhat elongated, is well fragmented in the transverse direction, the widest grain or grain fragment dimension being not over about 0.05 millimeter as measured in the transverse direction of the sheet at the conclusion of the controlled temperature rolling operations.

It has been found that the above-described alloy composition and hot-warm controlled rolling procedures which produce the described fragmented grain structure combine to produce a highly unique product, an economical architectural sheet capable of producing a rapidly developed integral anodic black color in existing anodizing equipment and procedures which sheet product can be bent without exhibiting incipient cracks, checking, kinks or any generally rough appearing surface condition thereby enabling the production of bent sheet shapes for architectural applications free of these defects which plagued previous products capable of approaching this type of color development. Furthermore, it has been found that the improved sheet product exhibits substantially complete freedom from structural streaking and, very significantly, greatly increased resistance to corrosion in polluted atmosphere thus providing for greatly improved and reduced maintenance costs on a completed building, especially a high-rise building which extends into the polluted atmospheres which seem to lurk above almost every site where large buildings are constructed.

The sheet product exiting the controlled warm rolling operation can typically range in thickness from 0.075 to 0.25 inches and is useful in these and other thickness with or without further processing. If desired, the sheet can be annealed in order to soften it for further working or forming operations. For instance, it can be fully an-

nealed at a temperature of around 600° to 700° F. and the sheet so treated exhibits less tensile strength but is easier to bend than in the condition as it exits the warm rolling operation. If desired the sheet product can be further worked as by cold rolling with or without first annealing. The strain hardening effects of cold rolling would confer higher strength to the sheet which may be desired in some instances. Additionally some amount of cold rolling can sometimes reduce any structural streaking problems in the anodized sheet product. The desirability of annealing before cold rolling would depend to some extent on the degree of the cold reduction.

One preferred embodiment of the invention contemplates providing the defined improved alloy as a cladding layer on an alloy core to provide a composite structure. This has the advantage of achieving a desired strength level from the core material while realizing the advantages of the invention in the cladding layer. A suitable core alloy is alloy 3003 which contains nominally 1.2% manganese and 0.12% copper, balance essentially aluminum. Thus the invention contemplates the use of such clad composites featuring the improved alloy as a cladding on one or both faces of a sheet produced and a core composed of an aluminum alloy which aluminum alloy may typically contain up to 2%, for instance 0.3 to 2% of manganese. This type of core alloy is highly compatible with the improved alloy with respect to rolling and other fabricating characteristics thus enabling relatively economical production of a clad product. When fabricating such a composite the cladding material in the improved alloy is fabricated into sheet according to the methods here described. This sheet is placed on one or both sides of the core rolling stock and hot roll bonded thereto to provide a bonded composite which is reduced by rolling. The rolling here does not need to proceed according to the improved controlled conditions since the cladding has already been previously broken down by the improved method.

The sheet product can be anodized to develop integrally colored anodic coatings. Employing an aqueous bath containing 130 to 200 grams per liter of sulfuric acid at a temperature of 70° to 90° F. and current density levels of 20 to 30 amps per square foot and maintaining anodizing conditions for 20 to 60 minutes a coating is produced ranging in thickness from about 0.7 to 1.2 mils and the coating exhibits an integral gold or yellow color. Using an aqueous bath containing about 95 grams of sulfophthalic acid and 5 grams of sulfuric acid per liter and maintained at temperatures of about 70° or 80° F. and current density levels of 25 to 30 amps per square foot a black integral anodic coating color is achieved within about 30 minutes. The black color is characterized by apparent reflectance and yellowness levels of less than 4% as determined by Color-Eye measurement. Again the coating is about 0.71 mil in thickness. Instead of sulfophthalic acid the electrolyte could contain one of the other sulfonic acids such as sulfosuccinic and sulfosalicylic acids.

It is usually desirable to seal the anodic coating, for example, by immersing in hot (210° F.) water or other suitable solutions. The coloration and texture developed in the anodic treatment can be modified by treatment of sheet prior to anodic oxidation. The surface can be chemically brightened by washing with a solution of phosphoric and nitric acids or electrochemical procedures. Mechanical treatments such as buffing, polishing, sand blasting and the like can also be employed to alter the texture of the surface prior to anodizing.

As indicated earlier the improved architectural sheet product when anodized exhibits improved resistance to corrosion thus rendering it highly suited for high-rise and other buildings such as in cities where polluted atmospheres may be present. In comparing different anodized sheet products an accelerated test has been developed which serves to indicate potential susceptibility to corrosion in highly polluted environments. Since the corrosion

occurs through the anodic coating and is dependent on weaknesses in the coating the test is directed to the coating. In this test, sample panels anodized under conditions described previously for developing integral black coatings on the subject alloy of this invention are immersed in a solution of 200 grams  $\text{CuSO}_4$  and 10 ml.  $\text{H}_2\text{SO}_4$  in 1 liter of water. A cathodic potential of 1.5 volts is applied for three minutes. By this procedure copper is deposited in any voids or holes in the anodic coating. In this test the improved sheet showed virtually no copper deposition which is indicative of a sound anodic coating of very high integrity and thus indicative of very good resistance to the corrosion effects of polluted atmospheres. On the other hand, panels of a commercial architectural sheet alloy, 6061 alloy containing nominally Al, 1% Mg, 0.6% Si, 0.25%, Cu and 0.2% Cr, used for integral color anodizing exhibited numerous spots of Cu deposition indicative of weak points in the coating thus leaving the anodized sheet quite susceptible to corrosion by atmospheric pollutants.

Example 1

A sheet product was fabricated from an alloy containing 0.47% Cu, 0.18% Fe, 0.07% Si, 0.17% Cr, 0.00% Mg, 0.02% Zn, 0.01% Ti, the balance aluminum. The alloy was continuously cast as an ingot which was homogenized at a temperature of 1100° F., cooled to room temperature in open air, scalped and then reheated to about 950° F. The scalped ingot was then introduced into a hot reversing mill at a conventional ingot metal temperature of 910° F. which reduced the thickness from about 12 inches to about 4 inches, a reduction of 67%. The 4-inch plate was then introduced to a second mill which reduced its thickness to about  $\frac{3}{4}$  inch. This plate was then run through a continuous mill at an entry temperature of about 650° F. which reduced its thickness to about  $\frac{1}{8}$  inch at an exit temperature of about 350° F. Sections of the sheet so produced were bent over a 4T radius (a radius of 4 times the sheet thickness) along a longitudinal direction and exhibited surface cracking, folds, and objectional kinking and checking along the bend radius. The bent sheet sections were anodized in the sulfophthalic-sulfuric acid aqueous anodizing bath described above for 30 minutes to develop an integral black coating. Metallographic examinations made of transverse sections through the bend areas revealed objectionable thinning of the anodic coating in localized areas as a consequence of irregular formation of the coating over the roughened surface which considerably diminished the integrity of the coating. The anodized bend area also exhibited visual defects including kinking and surface cracking or checking which, regardless of coating integrity, themselves are highly objectionable for architectural application.

Example 2

Improved sheet product was fabricated from an alloy containing 0.52% Cu, 0.22% Fe, 0.14% Si, 0.06% Mn, 0.007% Mg, 0.16% Cr, 0.025% Ti. The alloy was continuously cast as an ingot which was homogenized at a temperature of 1100° F., cooled to room temperature in open air, scalped and then reheated to a temperature of 800° F. The scalped ingot was then introduced into a hot reversing mill at an ingot metal temperature of 760-780° F. which reduced the thickness from about 14 inches to about 6 inches, a reduction of over 55%. The temperature exiting the mill was about 720° F. The 6-inch plate was then fed to a second mill which reduced its thickness to about 1 inch and the exit temperature of the second mill was about 650° F. The total hot reductions to this point amount to over 90% of the 14 inch thick starting stock. The 1-inch plate was then run through a hot continuous mill where it sustained an 80% reduction to produce a sheet approximately  $\frac{1}{8}$  inch in thickness at an exit temperature of about 350° F. Sections of this sheet were anodized in the sulfophthalic-sulfuric acid aqueous anodizing bath described above for 30 minutes

55  
60  
65  
70  
75

and the integral coating exhibited a jet black color characterized by apparent reflectance and yellowness values both under 4% as determined with the Color-Eye instrument. Sections of this sheet also were bent over a 1T radius along a longitudinal direction. This bend is four times more sharp, and hence more severe, than that mentioned in Example 1. Yet the specimens exhibited no incipient cracks, folds or objectionable checking along the bend radius. The bent sheet sections were anodized using the above-described conditions to develop the jet black color. Metallographic examinations made of transverse sections through the bend areas confirmed that the anodic coating was of very high integrity and further exhibited no visual defects.

What is claimed is.

1. A method of producing improved architectural sheet comprising the steps:

- (1) providing a body of aluminum base alloy consisting essentially of 0.4 to 0.6% copper, 0.1 to 0.25% chromium, 0.08 to 0.18% silicon, the balance aluminum and not more than the following amounts of other elements and impurities: iron 0.3%, manganese 0.05%, magnesium 0.1%, zinc 0.05%, titanium 0.05%, all other elements and impurities being limited to 0.05% each and a total of 0.1%, the amount of all elements other than aluminum, silicon, copper, chromium and iron not exceeding 0.2%.
- (2) homogenizing said body by heating it to a temperature within the range 1000° to 1150° F.,
- (3) hot rolling said body at temperatures which are controlled such that the metal temperature as it initially enters the rolling operation is between 600° and 800° F. and substantially avoiding metal temperatures in excess of 800° F. during rolling to produce a rolled product having a grain structure featuring a substantial amount of grain fragmentation across the long transverse direction.

2. A method of producing improved architectural sheet comprising the steps:

- (1) providing a body of aluminum base alloy consisting essentially of 0.4 to 0.6% copper, 0.1 to 0.25% chromium, 0.08 to 0.18% silicon, the balance aluminum and not more than the following amounts of other elements and impurities: iron 0.3%, manganese 0.05%, magnesium 0.1%, zinc 0.05%, titanium 0.05%, all other elements and impurities being limited to 0.05% each and a total of 0.1%, the amount of all elements other than aluminum, silicon, copper, chromium and iron not exceeding 0.2%.

- (2) homogenizing said body by heating it to a temperature within the range 1000° to 1150° F.,
- (3) rolling said body to reduce its thickness and alter its grain structure such that a substantial degree of grain fragmentation occurs in the long transverse direction, said fragmentation being initiated in the first rolling passes by avoiding in these passes metal temperatures in excess of 800° F., the body entering said initial roll passes at a metal temperature of between 600° and 800° F., to produce a rolled product having a fragmented grain structure such that the widest grain or grain fragment dimension in the long transverse direction does not exceed about 0.05 millimeter.

3. A method of producing improved architectural sheet comprising the steps:

- (1) providing a continuously cast body of aluminum base alloy consisting essentially of 0.4 to 0.6% copper, 0.1 to 0.25% chromium, 0.08 to 0.18% silicon, the balance aluminum and not more than the following amounts of other elements and impurities: iron 0.3%, manganese 0.05%, magnesium 0.1%, zinc 0.05%, titanium 0.05%, all other elements and impurities being limited to 0.05% each and a total of 0.1%, the amount of all elements other than alu-

- minum, silicon, copper, chromium and iron not exceeding 0.2%.
- (2) homogenizing said body by heating it to a temperature within the range 1000° to 1150° F.,
- (3) cooling said body at a cooling rate commensurate with open air cooling, and
- (4) hot-warm rolling said body to effect a reduction in its thickness of at least 40% at controlled temperatures, said rolling reducing the thickness and altering the cast internal structure of said body such that a substantial degree of grain fragmentation occurs in the long transverse direction, said fragmentation being initiated in the first rolling passes by avoiding in these passes metal temperatures in excess of 800° F. the body entering said initial roll passes at a metal temperature of between 600° and 800° F., said rolling proceeding without reheating the metal body, the metal temperature during said rolling decreasing but to a level not below 300° F., said rolling producing a rolled product having a fragmented grain structure such that the widest grain or grain fragment dimension in the long transverse direction does not exceed about 0.05 millimeter.
4. The method according to claim 2 wherein said rolled product is further reduced in thickness by cold rolling.
5. The method according to claim 1 wherein said alloy contains a controlled amount of magnesium of up to 0.1%.
6. The method according to claim 5 wherein the magnesium ranges from 0.005 to 0.05%.
7. The method according to claim 3 wherein the hot-warm reduction in said step (4) amounts to at least 80%.
8. The method according to claim 1 with the additional step of anodizing said rolled product to produce an integral colored anodic coating.
9. An improved architectural sheet product composed of an alloy consisting essentially of 0.4 to 0.6% copper, 0.1 to 0.25% chromium, 0.08 to 0.18% silicon, the balance aluminum and not more than the following amounts of other elements and impurities: iron 0.3%, manganese 0.05%, magnesium 0.1%, zinc 0.05%, titanium 0.05%, all other impurities being limited to 0.05% each and a

total of 0.1% the amount of all these elements and impurities other than aluminum, silicon, copper, chromium and iron not exceeding 0.2%, the sheet product exhibiting a substantial degree of grain fragmentation in the long transverse direction such that the largest grain or grain fragment size does not exceed about 0.05 millimeter in the long transverse direction as a result of controlled hot-warm rolling operations at temperatures of 300° or more but not to exceed 800° F., said sheet when bent to a radius of one time its thickness exhibiting substantial freedom from checks in the bend radius, said sheet further being characterized when anodized by the ability to develop an integral true black color said anodic coating having an improved level of resistance to attack by polluted atmospheres.

10. The improved sheet product according to claim 9 wherein said alloy contains a controlled amount of magnesium of up to 0.1%.

11. The improved sheet product according to claim 10 wherein the magnesium ranges from 0.005 to 0.05%.

12. The improved sheet product according to claim 9 wherein the sheet product features at least one bend of a radius one time its thickness or more and features an integrally bonded anodic coating having an integral black color characterized by maxima of 4% for yellowness and apparent reflectance.

#### References Cited

##### UNITED STATES PATENTS

|    |           |         |                  |            |
|----|-----------|---------|------------------|------------|
| 30 | 1,913,846 | 6/1933  | McCullough       | 75—143     |
|    | 2,941,930 | 6/1960  | Mostovych et al. | 148—11.5 A |
|    | 3,113,002 | 12/1963 | Hollingsworth    | 148—31.5   |
|    | 3,164,494 | 1/1965  | English          | 148—31.5   |
| 35 | 3,187,428 | 6/1965  | English          | 148—11.5 A |
|    | 3,370,943 | 2/1968  | Beatty           | 75—143     |

WAYLAND W. STALLARD, Primary Examiner

U.S. Cl. X.R.

40 148—11.5 A, 31.5, 32

UNITED STATES PATENT OFFICE  
CERTIFICATE OF CORRECTION

Patent No. 3,827,952 Dated August 6, 1974

Inventor(s) Edmund C. Franz

It is certified that error appears in the above-identified patent and that said Letters Patent are hereby corrected as shown below:

Col. 3, line 64                    Change "atmosphere" to --atmospheres--  
Col. 4, line 23                    Change "produced" to --product--  
Col. 5, line 68                    Change "65 $\Omega$ " to --650--

Signed and sealed this 12th day of November 1974.

(SEAL)

Attest:

McCOY M. GIBSON JR.  
Attesting Officer

C. MARSHALL DANN  
Commissioner of Patents